

Patented Feb. 8, 1927.

1,616,468

# UNITED STATES PATENT OFFICE.

FRIEDRICH RASCHIG, OF LUDWIGSHAFEN-ON-THE-RHINE, GERMANY.

## WOOD-PRESERVING COMPOSITION.

No Drawing. Application filed May 20, 1925, Serial No. 31,696, and in Germany February 13, 1925.

For many years dinitro-phenol and dinitro-cresol have been applied with good results to the preservation of wood, either in the nascent state or in the form of alkaline—  
5 or aniline salt (German Patent 219,893). Generally these nitro-combinations are applied in mixtures with large quantities of sodium fluoride.

But it has been proved, that these solutions  
10 strongly affect the vessels for holding the impregnation liquid. To prevent this inconvenience additions to the preserving composition have been proposed, for instance, the addition of potassium bichromate (German Patent 299,411), or the addition of compounds of the bi-valent metals, particularly  
15 of zinc (German Patent 368,490). Recently the application of antimonial salts has been recommended to prevent the attack upon iron  
20 by these solutions. But the opinions concerning the advantages of such additions are by no means agreed; it is said that an addition of bichromate for example favours the action upon the iron.  
25 I have discovered that aqueous solutions of sodium fluoride and dinitrophenol or dinitrocresol, which strongly affect iron not only in the cold state, but in a still higher degree in a heated state, immediately lose this prop-

erty, if a small quantity of water-glass is  
30 added. But this favorable result can not be explained by supposing, that the alkaline strength of water-glass saturates the dinitro-phenol to dinitrosodium phenolate, since an equivalent quantity of dinitrosodium phenolate in the mixture for impregnation does not show in the least degree the same favorable properties. Therefore, there is an effect, which is specific to the potassium or  
35 sodium silicate.

### Example.

88 parts sodium fluoride, 10 parts dinitrocresol, and 2 parts water-glass, finely powdered, are mixed together. The mixture is  
45 easily and completely dissolved in water; the solution does not attack iron even in the heated state.

I claim as my invention:

A wood-preserving composition consisting of 88 parts, by weight, of sodium fluoride; 10 parts, by weight, of dinitro-ortho-cresol; and 2 to 10 parts, by weight, of water-glass.

In testimony whereof I have affixed my  
signature.

FRIEDRICH RASCHIG.